

## UNITED STATES PATENT OFFICE

1,938,456

GUM INHIBITING TREATMENT OF CRACKED  
PETROLEUM DISTILLATESHerman P. Lankelma, Cleveland, Ohio, assignor  
to The Standard Oil Company, Cleveland, Ohio,  
a corporation of OhioNo Drawing. Original application August 7, 1930,  
Serial No. 473,774. Divided and this applica-  
tion February 20, 1933. Serial No. 657,685

6 Claims. (Cl. 44—9)

This invention relates to the preparation of stable products from cracked petroleum distillates, and more particularly from cracked naphthas for motor fuels. As now well known, cracked 5 distillates inherently tend to develop more or less gum formation and also go off color. It is among the objects of the invention to inhibit such detrimental tendencies in cracked distillates, and in a manner which can be carried out 10 without material disarrangement of desirable practice generally.

To the accomplishment of the foregoing and related ends, the invention then, consists of the features hereinafter fully described, and particularly pointed out in the claims, the following description setting forth in detail certain embodiments of the invention, these being illustrative however, of but a few of the various ways in which the principle of the invention may be 20 employed.

In accordance with my invention, a cracked petroleum distillate such as is prone to develop gum formation is subjected to the action of an acyl derivative of an amino-phenol, that is, an 25 amino-phenol in which at least one amino-hydrogen atom is substituted by a radical from the group of acyls, such for instance as acetyl-amino-phenols, and in a specific illustration para-acetyl-amino-phenol.

30 One or more of these agents is incorporated in the cracked distillate to be treated. The amount of such agent required is small, for instance, 0,0004 to 0,5 per cent. In general therefore, it is not necessary to exceed one-half of one per 35 cent, or at the outside one per cent, amounts thereover being wasted. A desirable manner of incorporating the material into the petroleum distillate may involve first dissolving the agent in a suitable solvent, as for instance ether, benzol, 40 or the like, and such solution may then be mixed with the distillate. The petroleum distillate may have been previously subjected to a customary lye wash if desired, and in fact a slight alkaline or at least neutral reaction of the distillate is 45 advantageous. The mixing may be effected in any convenient manner, as for instance adding the agent to the petroleum in a container and suitably agitating to a good dissemination, or proportionally feeding into a flowing stream of 50 the petroleum in calibrated amount.

Example.—20 pounds of para-acetyl-amino-phenol is dissolved in a desired amount of benzol and this in turn is mixed with 2500 barrels of cracked gasoline.

55 Similarly as indicated, any of the various

agents contemplated can be incorporated, and cracked distillates be so treated, with the production of motor fuels and the like, which may be successfully stored and used, with control of the gumming and discoloration tendencies otherwise prone to occur.

This application is a division of my application Serial No. 473,774, filed August 7th, 1930.

Other modes of applying the principle of the invention may be employed instead of the details disclosed, change being made as regards such details, provided the features stated in any of the following claims, or the equivalent of such, be employed.

I therefore particularly point out and distinctly claim as my invention:—

1. A volatile cracked petroleum distillate treated with a small amount of an acyl-substituted amino-phenol.

2. A volatile cracked petroleum distillate 75 treated with a small amount of an acetyl-amino-phenol.

3. A volatile cracked petroleum distillate treated with a small amount of para-acetyl-amino-phenol.

4. A process of treating a cracked petroleum distillate, which comprises subjecting such distillate to the action of a small amount of an acyl-substituted amino-phenol.

5. A process of treating a cracked petroleum 85 distillate, which comprises subjecting such distillate to the action of a small amount of an acetyl-amino-phenol.

6. A process of treating a cracked petroleum distillate, which comprises subjecting such distillate to the action of a small amount of para-acetyl-amino-phenol.

HERMAN P. LANKELMA.

95

100

105

110